# EUROPEAN PATENT SPECIFICATION

(11) **EP 0 046 209 B1**
(45) Date of publication and mention of the grant of the patent: **10.09.1986**
(21) Application number: 81105783.5
(22) Date of filing: 22.07.1981
(51) Int. Cl.: B22F 7/06, C22C 1/05, C22C 29/00, B23B 27/14

(54) **Steel-hard carbide macrostructured tools, compositions and methods of forming**
Grobstrukturierte Werkzeuge, bzw. Werkstoffe, aus Stahl-Hartkarbiden und Herstellungsverfahren
Outils et compositions ayant une structure macroscopique acier-carbure dur et leur procédé de fabrication

(30) Priority: 18.08.1980 US 178805; 20.04.1981 US 255453
(43) Date of publication of application: 24.02.1982
(73) Proprietor: KENNAMETAL INC., Latrobe Pennsylvania 15650 (US)
(72) Inventor: Makrides, Nicholas, Delmont, Pennsylvania 15626 (US); Stoll, William Max, Ligonier Pennsylvania 15658 (US)
(74) Representative: Leiser, Gottfried, Dipl.-Ing.

## Description

### Background of the Invention

Since 1940, wear-resistant parts for wear-prone tools and equipment have been made of cemented carbide alloys consisting of a finely- dispersed hard-carbide phase based on metals chosen from Groups IVB, VB and VIB of the Periodic table, cemented by cobalt or nickel or both. Produced by compacting finely-milled powders followed by liquid-phase sintering to achieve consolidation, cemented carbide alloys possess micro-structures characterized by hard carbide grains generally in the 1 to 15 micron range.

The use of iron or steel as binder materials has proven difficult because the finely-divided state and high specific surface of the dispersed hard phases promote the formation of comparatively brittle binary interstitial alloys of tungsten and iron with carbon, thus reducing the free binder volume fraction and embrittling the sintered body, more or less, depending on the precision maintained in the formulation and sintering parameters and on the free carbon additions made to satisfy the affinity between iron and carbon.

Unlike cobalt and nickel, iron forms a stable carbide, Fe₃C, and has a greater tendency to form brittle binary carbides than cobalt or nickel binder materials. Carbon transfer from the hard carbide phase or phases to iron is promoted by the presence of the liquid or plastic state of an iron or steel binder during liquid-state sintering, carried out at temperatures near to, at, or above the melting point of the binder.

More recently, useful wear parts have been made by casting a liquid steel or cast iron melt into a prepared bed of comparatively coarse particulate, e.g. 3.175 to 4.763 mm sintered, cemented carbide.

CH-A-215 453 discloses a composition of matter comprising at least 80% of a carbide material selected from the group consisting of tungsten carbide and mixtures of tungsten carbide with other carbides such as titanium carbide, tantalum carbide, niobium carbide or vanadium carbide, and 20% maximum of an auxiliary metal such as cobalt, nickel and/or iron. Besides, said reference is concered with cemented carbide tools consisting of a base of sintered alloy such as nickel-iron, iron-chromium-tungsten alloy or molybdenum alloy.

GB-A-530 639 teaches a process of producing tools having supporting bodies provided with insets of hard metal with the insets being molded from a powdered mixture of carbides, borides, nitrides, and the like of a metal of the tungsten group, and of a binding metal which preferably consists of the same metal of which the supporting body is made, namely iron, steel, and other metals of the iron group.

The present invention may be distinguished from the molten-steel casting method of Charles S. Baum, US-A-Nos. 4,024,902 and 4,140,170 and the molten-cast iron method of Sven Karl Gustav Ekemar in US-A-4,119,459 by two main factors: (1) a powder compact of steel or iron and graphite containing dispersed particulates or sintered, cemented carbide, or a number of pieces of dimensioned sintered cemented carbide, or primary, unmilled macrocrystalline carbide crystals is sintered at a temperature below the melting temperature of steel or cast iron, and (2) in place of the use of matrix-alloy melting temperatures to achieve alloy densification, high compaction unit pressures, both before and after sintering, are used, thereby avoiding degradation of the dispersed hard phase particle surfaces by decomposition, melting or carbon diffusion reactions.

Foundry methods, also, lack tha well-known economic advantages inherent in powder metallurgy methods, notably, when a multiplicity of wear parts either small or of thin section are to be made. Also, because of the necessarily relatively high processing temperatures and liquidity, excessive amounts of unwanted binary carbides may form despite the use of comparatively coarse, low-surface area carbide particles.

Since both the conventional powder metallurgy method of pressing and sintering finely-milled steel-cemented carbide powders and methods involving casting liquid steel or liquid cast iron into particulate cemented carbide prearranged in molds result in problems hereinbefore described, it is the primary objective of this invention to develop a method by which a steel-cemented hard carbide alloy can be fabricated essentially free of binary interstitial alloys of iron and tungsten with carbon and in which the dispersed hard carbide phase is free of boundary-area decomposition, melting or thermal cracking and is firmly bound in a steel matrix essentially free of macroporosity.

It is also an object of this invention to produce a composite wear resistant body having dispersed hard carbide material firmly and adherently bonded in a metallic matrix by powder metallurgical techniques of compaction and high temperature and high pressure diffusion bonding as well as to provide a method for manufacturing said composite wear resistant body.

It is a further object of this invention to manufacture tools having hard carbide wear or cutting inserts embedded in and bonded to a consolidated steel powder matrix or composite wear resistant body according to this invention.

It is a further object of this invention to manufacture parts being substantially nonmachinable and of sufficient impact resistance to make them suitable for use as security plates and padlock components.

### Brief Summary of the Invention

This invention provides a solid-state sintered steel hard carbide composite wear resistant body comprising:
30 to 80 weight percent of a carbide material having a size greater than 37 um; said carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions, and their cemented composites; 20 to 70 weight percent of a matrix material selected from the group consisting of steel, steel and iron, steel and copper, and steel and nickel; said carbide material embedded in and bonded to said matrix; and an interface between said carbide material and said matrix no greater than 50 microns in thickness, said interface being essentially free of brittle double carbides.

In a preferred embodiment of the invention, the said carbide material additionally has a metallic coating forming a tough and adherent bond between said carbide material and said matrix.

The method of the present invention for manufacturing the said composite wear resistant body involves blending and mixing sintered, cemented tungsten carbide particles or primarily unmilled macrocrystalline (i.e., greater than 37 pm) tungsten carbide crystals with a matrix of iron and graphite powders or steel powder, cold isostatically pressing the composite in a preform mold to a desired shape, then solid-state sintering at a comparatively low temperature, specifically, at a temperature below the melting temperature of the steel, preferably, between 1038°C and 1232°C, then hot isostatically solid-state pressing (HIP) the sintered body at a temperature well below the melting point of steel to achieve final densification. A diffusion body is formed between the hard carbide particles and the surrounding steel powder, which holds the wear-resistant hard carbide particles in place.

Furthermore, the present invention is concerned with a tool made by the same method according to the invention comprising: a working end having a hard wear resistant cemented carbide insert; a body having steel; a bond region joining said insert to said body; characterized in that said bond region comprises an alloy having iron and cobalt and being essentially free of brittle double carbides of iron and tungsten.

And finally, this invention is concerned with the use of said method for forming said cemented carbide tool comprising embedding a predimensioned cobalt cemented carbide insert in a predetermined Icoation in a blend of steel forming powder; consolidating said powder around said insert to form a preform; and interdiffusing cobalt from said insert with iron from said consolidated steel forming powder adjacent the insert at a high temperature below the temperature at which the steel is at least partially liquid and, simultaneously at a high pressure, to form a metallurgical bond between said insert and said steel.

A critical factor of the present invention is high-pressure densification, both cold and hot, to avoid process temperatures which produce liquidity of the steel binder phase and, thus, promote the aforementioned undesirable reactions between the steel binder material and hard dispersed phase. The technique is reinforced in this respect by the use of a hard dispersed particle or particles of low specific surface. The method also provides a significant advance in production capability small size or of thin section or intricate design, as compared with methods as disclosed in United States patents hereinbefore enumerated in which molten steel or molten cast iron are poured into a mold preloaded with particles or cemented carbide.

Further, both chemical control of and compositional flexibility of the matrix alloy are superior to molten-metal casting methods. The avoidance of high processing temperatures required to melt and pour steel or cast iron provides better economy of molds, which may be reused, and matrix metals, which are not subject to pouring loss and recycle cost. The method of the present invention is well suited for the formation of parts that must withstand highly abrasive wear forces as well as impact forces. The process is ideally suited to form wear-resistant parts and cutting tools for equipment for agriculture, road and highway construction and maintenance, crushing, comminuting, excavation, and processing. Since the wear resistance of the products produced by this process is so high, so as to make them practically nonmachinable, they are also ideally suited for use as security plates in safes. This wear resistance in combination with the impact resistance of these compositions makes then also suitable for use in padlocks.

### Brief Description of the Drawings

The exact nature of the present invention will become more clearly apparent upon reference to the following detailed specification taken in connection with the accompanying drawings in which:
Figure 1 is a photomicrograph at 1500 magnification showing a cemented carbide particle having a cobalt binder embedded in and bonded to a consolidated steel powder matrix.
Figure 2 is a cross sectionalized perspective view of a wear plate having cemented carbide inserts embedded in and bonded to a consolidated steel powder matrix.
Figure 3 is a cross sectional view of part of a cutting tool having cemented carbide button embedded in and bonded to a consolidated steel powder matrix.

### Detailed Description of the Invention

Prealloyed steel matrix powder, or a mixture of iron powder and graphite powder, comprising 20 weight per cent (w/o) to 70 w/o of the final mixture is blended and mixed with 30 w/o to 80 w/o of hard carbide particles of W, Ti, Ta, Nb, or Zr, V, Hf, Mo, B, Si, Cr or a mixture of these, either as sintered cemented carbide particles or as primary, uncemented, unsintered, unmilled carbide crystals. About 3 percent of naphtha or other liquid hydrocarbon is added to the powder blend during mixing to prevent segregation of higher density carbide particles during mixing and mold filling, specifically when the dispersed hard phase is composed of hard carbide particles coarser than about 250 microns.

For dispersed hard phase particles finer than about 250 microns, paraffin wax or a solid lubricant such as zinc stearate may be used, because the possibility of component particle segregation during mixing is then diminished.

Next, the matrix powder containing the dispersed hard carbide phase is packed in a preform mold made of polyurethane or other elastomeric plastic. Steel powders of different chemical compositions (such as carbon, alloy or stainless steel powders) or elemental powders such as iron, copper or nickel, may also be packed in the same mold with the main composite steel powder- carbide blend, in any desired location, adjacent to and in contact with the body containing the hard carbide dispersed phase, or surrounding such body, or enveloping a dimensioned, sintered cemented carbide insert. The packed mold with a suitable fitted cover is then sealed and placed in a rubber bag or balloon which is then evacuated, sealed and isostatically pressed, preferably at about 2,413.25.10⁵ Pa, but not less than 689.5,10⁵ Pa.

The compacted powder preform is then removed from the mold and heated in vacuum or in a protective or reducing gas atmosphere, e.g., hydrogen, to a temperature below the melting temperature of the steel matrix, preferably between 1038°C and 1149°C, for between 20 and 90 minutes.

An alternative preforming method consists of packing the composite mixture containing preferably liquid hydrocarbon, e.g. naphtha, preferably 7 w/o and methyl cellulose, preferably 0.5 w/o, as pressing lubricant and green-state binder, respectively, in a steel preform mold. The green preform is then air dried at room temperature, in the mold, then removed from the mold and placed in a rubber bag which is then evacuated and sealed, ready for cold isostatic compaction as hereinbefore described.

Compacts thus solid-state sintered retain some porosity; shrinkage during sintering does not exceed 1 per cent. It has been found, however, that densification achieved by high-pressure isostatic compacting followed by sintering as herein described is sufficient to eliminate any interconnected pore network and that the sintered bodies, therefore, qualify for effective final densification by known hot isostatic pressing (HIP) methods.

Hot isostatic pressing for the purpose of this invention is applied in an inert atmosphere, preferably at 871°C to 1260°C or at any temperature below the melting temperature of the steel for from 20 to 90 minutes at a minimum pressure of 689.5-10⁵ Pa but, preferably at a pressure of about 1,034.25-10⁵ Pa for 60 minutes. Equally important, an alloy layer is formed at the interfaces of cemented carbide particles and steel matrix. This interfacial alloy bond, which first forms during sintering and is later enhanced during hot isostatic pressing, consists of a thin border area between, for example, a 0.75 per cent carbon steel matrix and dispersed cobalt-cemented carbide particles in a 3.175 to 4.763 mm size range. The bond is typically less than 40 microns thick, and no greater than 50 microns thick. The interfacial bonding alloy under these conditions is composed of, principally, cobalt and iron. Bond formation becomes important especially when the hard dispersed phase is of comparatively coarse particles, because these are apt to pull out if not securely anchored in the matrix alloy.

Cemented tungsten carbide particle sizes comprising the dispersed hard phase are selected from within the general size range of 8 mm to 0.149 mm (2.5 mesh to 100 mesh in the U.S. sieve series), preferred size ranges being of from 0.84 to 1.53 mm (+20 to -12 mesh), from 1.53 to 3.36 mm (+12 to -6 mesh), and from 3.36 to 4.76 mm (+6 to -4 mesh). Specific selected size ranges may be prepared by known methods of crushing and sizing sintered, cemented carbide tool components, and which alloys are more commonly of a cobalt or nickel-cemented tungsten carbide (WC) base, sometimes containing also TiC, TaC or NbC or combinations of these hard carbides.

An additional useful aspect in the process of the present invention is to apply a coating of an alloy or metal, preferably Corson bronze or nickel, on the surfaces of a dimensioned sintered cemented tungsten carbide insert of selected shape and size, or a number of such inserts, which are then embedded in a steel or iron-graphite matrix powder at selected locations within a preform mold before the filled mold is isostatically compacted. The corson bronze coating used may be either of the two nominal compositions shown in Table I.

Following cold isostatic compaction and during subsequent sintering and hot isostatic pressing of the carbide-steel compact, the coating on the cemented carbide body autogenously forms a diffusion bond, to increase the bonding strength with which dimensioned cemented carbide bodies are held in the matrix. By this method, a cemented carbide body, or a number of them, of specific shape and size may replace a dispersed hard carbide phase of particulate nature, and thereby form a wear-resistant body or a tool for cutting or drilling metal or rock.

It is recognized that the comparatively low processing temperatures employed in the process of this invention may, in cases in which steel matrix powder compositions are used which do not bond well to particles of a dispersed hard carbide phase, result in inadequate bond strength at the matrix-carbide particle interface. In such cases, for example when alloy steel powders are used which are known to be less sinterable at the comparatively low solid-state sintering temperatures described in the process of this invention, it has been found beneficial to precoat the hard carbide particles with nickel or copper, for example, by known processes such as electroless metal coating or by cacuum vapor-phase coating. Nickel coatings thus applied to the hard carbide dispersed fraction, prior to blending, have been found to improve carbide particle bonding strength. Such precoating of the hard carbide particles would also be beneficial when stainless steel powders are being used.

A further and useful part of the foregoing method is the incorporation of a dispersed hard carbide phase in a steel or iron-graphite powder compact consisting of unmilled macrocrystalline carbide crystals in size range fractions between 0.037 and 0.250 mm (betweeen 400 and 60 mesh) and in preferred size ranges of e.g. from 0.149 to 0.250 mm (+100 to -60 mesh), from 0.074 to 0.177 mm (+200 to -80 mesh), or from 0.044 to 0.099 mm (+325 to -150 mesh), instead of and in place of particles of cemented carbide. The method of the present invention for formulating and forming macrostructred cemented carbide compositions is exactly as heretofore described.

The relatively low processing temperature practiced results in a macrostructure essentially free of brittle double carbides of iron and tungsten (eta phase) and gross porosity. The tendency for liquid-phase sintered, microstructured, cemented tungten carbide alloys employing a steel binder, for example, in place of the usual cobalt binder, to develop brittle eta-type phases is well known. It is believed that the avoidance of liquid phase sintering and consequently the avoidance of carbon- transfer that such practice encourages, as well as the uniquely low specific surface of the unmilled macrocrystalline carbide particles comprising the dispersed hard phase are essential for the successful formation of the two-phase, steel-carbide macrostructures produced by this method. It should be understood that liquid phase sintering as referred to herein means sintering at a temperature at which the steel binder is at least partially liquid. The prohibition of liquid phase sintering in this invention, therefore, does not apply to any lower melting point metals or alloys (e.g., copper or corson bronze) which may be added as a powder or coating to promote bonding or densification, and may intentionally become liquid during sintering or hot isostatic pressing.

The use of unmilled macrocrystalline hard carbide crystals as a dispersed hard phase is a preferred embodiment of the method of this invention, as an efficient means of maintaining a hard phase possessing low specific surface. It is recognized, however, that essentially binderless, hard aggregates of finer or milled hard carbides may be so used.

An important aspect of the aforementioned macrostructured bodies is the avoidance of ball milling or other comminution of the matrix-carbide powder mixtures, or of either of these two materials separately, prior to cold isostatic compaction, sintering and HIP. The former practice, widely considered essential to sound commercial cemented carbide structures, leads to enhanced reaction between carbides and iron-base matrix powders with resultant formation of brittle double carbides. Avoidance of powder milling also reduces cost.

The method of the invention may employ any of the macrocrystalline carbides, or combinations or solid solutions of them, specifically WC, TiC, TaC or NbC, all exhibiting the low specific surface and angular, blocky shapes typifying these coarsely-crystalline mono and binary carbides. It is known that primary macrocrystalline carbide materials may be finely milled, together with cobalt or nickel, to form cemented carbide micro-structures by liquid-phase sintering in the temperature range 1316°C to 1538°C, in which the resultant dispersed hard carbide phases are typically between one micron and about ten microns. The method of the invention, in contast, results in dispersed, single macrocrystalline carbide grains in size ranges selected from within the much coarser extremes of 250 microns to about 40 microns.

This invention is further explained by the following examples:

### Example No. 1

Wear resistant cutting tips were fabricated for rotary sugar cane shredding machines. A uniformly blended mixture composed of approximately 55 w/o 3.175 to 4.763 mm cobalt cemented tungsten carbide granules, approximately 44.67 w/o to less than 0.149 mm atomized iron powder and 0.33 w/o of smaller than 0.044 mm graphite powder was prepared. During blending 5 w/o of naphtha was added to minimize segregation of the higher-density cemented carbide particles. The dample mixture was manually compacted into an elastomeric polyurethane mold cavity of the desired tool shape, dimensioned to allow for cold isostatic powder compaction plus one per cent sintering shrinkage. Following cold isostatic compaction at 2,413.25.10⁵ Pa, the compacted preform was removed from the mold and vacuum sintered at 1093°C for 60 minutes, following which the sintered body was isostatically pressed at 1232°C for 60 minutes at 1,034.25·10° Pa under helium.

Metallographic examination disclosed a matrix structure composed of mostly pearlite and a little ferrite typical of conventional slow-cooled 0.75 per cent carbon steel of low porosity. The cemented carbide-matrix interfaces were occupied by bands of a width of about 5 microns of an alloy believed to be composed of iron and cobalt, principally. The cemented carbide dispersed particles appeared unimpaired by thermal cracking and no evidence of dissolution, melting or decomposition of the dispersed carbide phase existed at or near the interfacial boundaries, such boundaries being sharp except for the aforementioned iron-cobalt alloy diffusion zone. No potentially harmful concentrations of eta phase were observed. Test bodies were manually bent over a mandrel by hammering at room temperature and found to have a high resistance to impact loading and to be essentially free of brittle fracture.

Figure 1 is a photomicrograph of a typical area in a composite produced according to Example 1, except that sintering was done at 1149°C. A cobalt cemented tungsten carbide granule 40 is shown metallurgically bonded to a plain carbon steel having a mostly pearlitic structure 50 by a diffusion zone 45 containing iron and cobalt. The diffusion zone 45 is approximately 3 microns thick.

### Example No. 2

A wear-resistant, 12.9 cm² by 0.95 cm thick plate was fabricated consisting of 60 w/o of unmilled macrocrystalline WC having a particle size of from 0.149 to 0.250 mm (+100 to -60 mesh) and being cemented by 40 w/o of 0.75 per cent C steel containing 2 w/o Cu. A uniformly dry blended mixture of macrocrystalline WC crystals having a particle size of from 0.149 to 0.250 mm (+100 to -60 mesh), graphite powder having a particle size of less than 0.044 mm (-325 mesh), iron powder of less than 0.149 mm (-100 mesh), and copper powder of less than 0.044 mm (-325 mesh) were dry blended, unmilled, to a uniform mixture, then dampened by blending with liquid naphtha and methyl cellulose equal, respectively, to 7 per cent and 0.5 w/o of the dry mixture, and then packed into a steel preform mold to a firm, green, plate shape of dimensions equal to approximately 102 per cent of the desired final dimension.

Following air drying in the mold at room temperature, the compact was removed from the mold, placed in a rubber bag and further processed by cold isostatic compaction, sintering and HIP as described in Example No. 1. Metallographic examination revealed a macrostructure of macrocrystalline WC evenly dispersed throughout a steel matrix. A 5 micron thick bond layer of unknown composition was observed at WC-steel interfaces.

These interfaces were free of brittle binary carbide phases and cracks.

### Example No. 3

A composite 38.1 mm cubic wear-resistant body of steel enclosing a dimensioned plate of sintered, cemented 5 w/o cobalt-tungsten carbide was fabricated, purposefully embedding the dimensioned plate of sintered, cemented carbide in the green powder prior to iso-compaction so that its outer surface was flush with the outer surface of the steel cube. A dry unmilled blend comprised of 97.25 w/o to less than 0.149 mm (-100 mesh) atomized iron powder, 2 w/o less than 0.044 mm (-325 mesh) Cu powder and 0.75 w/o graphite was made, then blended with naphtha and methyl cellulose equal to, respectively, 5 w/o and 0.3 w/o of the dry blend. This was then packed into an elastomeric mold following which a 25.4 mm square by 6.35 mm thick plate of sintered cemented carbide was pressed down into the iron powder mix so that the outer surfaces were congruent.

The mold, after sealing, was placed in a rubber bag, evaculated, sealed and at this point was isostatically compacted, removed from the mold, sintered and hot isostatically compacted as in Example No. 1. Metallographic examination revealed that the prepositioned sintered carbide plate was bonded by a 5 micron interfacial bond phase to the steel matrix surrounding it on three sides and that the entire structure appeared sound and free of cracks.

Figure 2 presents a description of a wear plate 20 manufactured in the manner described in this example, except that three rather one cemented carbide inserts 30 are embedded in the plate 20 such that a surface 45 of each insert 30 is substantially flush with the working end 40 of the tool 20. It will be noted that the interfacial bond 35 is substantially uniform and continuous and forms a tough and adherent bond between the cemented carbide and the consolidated carbon steel and copper matrix 25.

In certain wear applications, depending on the corrosion nature of the environment in which the wear plate will be used, stainless steel or alloy steel powders may be advantageously substituted for the iron, carbon and copper powders utilized in this example.

Figure 3 provides a cross sectional view of another embodiment of a tool according to the present invention. This tool 1 can be manufactured substantially as described in Example 3, except that the cemented carbide insert 5 is allowed to have its working end 2 extend outward and beyond the steel body 10 of tool 1. As shown in this figure, the insert 5 bonded to the steel body 10 by a diffusion zone 15 which was formed by the interdiffusion of cobalt from the insert 5 and iron from the steel body 10 during high temperature and high pressure sintering operations.

Modifications may be made within the scope of the appended claims.

## Claims

1. A solid-state sintered steel hard carbide composite wear resistant body comprising: 30 to 80 weight percent of a carbide material having a size greater than 37 um; said carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions, and their cemented composites; 20 to 70 weight percent of a matrix material selected from the group consisting of steel, steel and iron, steel and copper, and steel and nickel; said carbide material embedded in and bonded to said matrix; and an interface between said carbide material and said matrix no greater than 50 um in thickness, said interface being essentially free of brittle double carbides.

2. Body according to Claim 1 further characterized in that said interface has a thickness of 0 to 40 um.

3. Body according to Claim 1 wherein said carbide material is a cemented composite having a cobalt binder; and further characterized in that said interface has iron and cobalt and a thickness of 0 to 40 pm.

4. Body according to Claim 3 further characterized in that said cemented composite contains tungsten carbide.

5. Body according to Claim 1 further characterized in that said hard carbide is tungsten carbide.

6. Body according to Claim 1 further characterized in that said body is ductile at room temperature.

7. Body according to Claims 1, 3 or 5 further characterized in that said steel is an alloy steel.

8. Body according to Claims 1, 3 or 5 further characterized in that said steel is a stainless steel.

9. A solid-state sintered steel hard carbide composite wear resistant body comprising: 30 to 80 weight percent of a carbide material having a size greater than 37 pm and having a metallic coating; said carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions and their cemented composites; 20 to 70 weight percent of a matrix material selected from the group consisting of steel, steel and iron, steel and copper, and steel and nickel; and said metallic coating forming a tough and adherent bond between said carbide material and said matrix.

10. Body according to Claim 9 further characterized in that said steel is selected from the group consisting of alloy steels and stainless steels.

11. A body according to any one of claims 1 to 10 comprising: 30 to 80 weight percent of a carbide material having a size greater than 37 pm; said carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions and their cemented composites; 20 to 70 weight percent of a matrix material selected from the group consisting of steel, steel and iron, steel and copper, and steel and nickel; characterized in that said carbide material is embedded in and bonded to said matrix by powder metallurgical techniques of compaction and solid state diffusion bonding.

12. A method for manufacturing the steel hard carbide composite wear resistant bodies according to any one of claims 1 to 8 and 11 comprising: blending 20 and 70 weight percent of steel forming powders with 30 to 80 weight percent of hard carbide particles having a particle size between 8 mm and 37 um to produce a mixture; said steel forming powders selected from the group consisting of iron and graphite, alloy steels and stainless steels; said hard carbide particles selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions and their cemented composites; cold pressing said mixture to produce a compacted preform; and solid-state densifying said compacted preform via a high temperature and high pressure diffusion bonding and sintering process comprising solid-state sintering said compacted preform at a temperature above 1038°C and below the solidus temperature of said steel to minimize interconnected porosity in the preform and then hot isostatically solid-state pressing said preform at a pressure above 689.5-10⁵ Pa and a temperature between 871°C and the melting temperature of the steel.

13. A method according to claim 12 for manufacturing the steel hard carbide composite wear resistant bodies according to any one of claims 9 to 11 further characterized by coating said hard carbide particles with a metallic coating prior to said blending with said steel forming powders.

14. A tool made by the method of claim 12 or 13 comprising: a working end having a hard wear resistant cemented carbide insert; a body having steel; a bond region joining said insert to said body; characterized in that said bond region comprises an alloy having iron and cobalt and being essentially free of brittle double carbides or iron and tungsten.

15. A tool made by the method of claim 12 or 13 comprising: a working end having a hard wear resistant cobalt cemented carbide insert; a body having steel; said insert powder metallurgically bonded to said body by a diffusion zone formed during high temperature solid-state sintering below the melting point of said steel; and said diffusion zone having iron and cobalt and being essentially free of brittle double carbides of iron and tungsten.

16. A tool made by the method of claim 12 or 13 comprising: a working end having a hard wear resistant cemented carbide insert; said insert comprising 30 to 80 weight percent of a carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions and their cemented composites, and 20 to 70 weight percent of a matrix material selected from the group consisting of steel, steel and iron, steel and copper, and steel and nickel; a body having steel; said insert powder metallurgically bonded to said body by a diffusion zone formed during high temperature solid-state sintering below the temperature at which the steel binder is at least partially liquid; said diffusion zone being essentially free of brittle double carbides of iron and tungsten.

17. Use of the method of claim 12 or 13 for forming the cemented carbide tool according to claim 14 or 15 characterized by embedding a predimensioned cobalt cemented carbide insert in a predetermined location in a blend of steel forming powder; consolidating said powder around said insert to form a preform; and interdiffusing cobalt from said insert with iron from said consolidated steel forming powder adjacent the insert at a high temperature below the temperature at which the steel is at least partially liquid and, simultaneously at a high pressure, to form a metallurgical bond between said insert and said steel.

18. Use of the method of claim 12 or 13 for forming the cemented carbide tool and claim 16 comprising: embedding a predimensioned cemented carbide insert in a predetermined location in a blend of steel forming powder; said predimensioned cemented carbide insert comprising 30 to 80 weight percent of a carbide material selected from the group of hard carbides consisting of tungsten carbide, titanium carbide, tantalum carbide, niobium carbide, zirconium carbide, vanadium carbide, hafnium carbide, molybdenum carbide, chromium carbide, boron carbide, silicon carbide, their mixtures, their solid solutions and their cemented composites, and 20 to 70 weight percent of a matrix material selected from the group consisting of steel, steel and iron, steel and copper, and steel and nickel; consolidating said steel forming powder around said predimensioned insert to form a preform, solid-state sintering said preform at a temperature in the range of from 1038 to 1232°C and simultaneously at a pressure above 689.5,10⁵ Pa to form a metallurgical bond between said insert and said steel.

## Patentansprüche

1. Verschließfester, in festem Zustand gesinterter Stahl-Hartcarbid-Verbundkörper, umfassend: 30 bis 80 Gew.% eines Carbidmaterials mit einer Teilchengröße von mehr als 37 pm, wobei das Carbidmaterial aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählt ist; 20 bis 70 Gew.% eines der aus Stahl, Stahl und Eisen, Stahl und Kupfer, und Stahl und Nickel bestehenden Gruppe ausgewählten Matrixmaterials, wobei das Carbidmaterial in die Matrix eingebettet und an diese gebunden ist; und eine nicht mehr als 50 pm dicke Zwichenschicht zwischen dem Carbidmaterial und der Matrix, wobei die Zwischenschicht im wesentlichen frei von spröden Doppelcarbiden ist.

2. Körper nach Anspruch 1, ferner dadurch gekennzeichnet, daß die Zwischenschicht eine Dicke von 0 bis 40 um besitzt.

3. Körper nach Anspruch 1; dadurch gekennzeichnet, daß das Carbidmaterial ein zementierter Verbund mit einem Kobalt-Binder ist und daß die Zwischenschicht Eisen und Kobalt enthält und eine Dicke von 0 bis 40 um aufweist.

4. Körper nach Anspruch 3, ferner dadurch gekennzeichnet, daß der zementierte Verbund Wolframcarbid enthält.

5. Körper nach Anspruch 1, ferner dadurch gekennzeichnet, daß das Hartcarbid Wolframcarbid ist,

6. Körper nach Anspruch 1, ferner dadurch gekennzeichnet, daß der Körper bei Raumtemperatur duktil ist.

7. Körper nach einem der Ansprüche 1, 3 oder 5, ferner dadurch gekennzeichnet, daß der Stahl ein Legierungsstahl ist.

8. Körper nach einem der Ansprüche 1, oder 5, ferner dadurch gekennzeichnet, daß der Stahl ein nichtrostender Stahl ist.

9. Verschleißfester, in festem Zustand gesinterter Stahl-Hartcarbid-Verbundkörper, umfassend: 30 bis 80 Gew.% eines Carbidmaterials mit einer Teilchengröße von mehr als 37 um und mit einem metallischen Überzug, wobei das Carbidmaterial aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählt ist; 20 bis 70 Gew.% eines der aus Stahl, Stahl und Eisen, Stahl und Kupfer, und Stahl und Nickel bestehenden Gruppe ausgewählten Matrixmaterials, wobei der metallische Überzug eine zähe und festhaftende Bindung zwischen dem Cärbidmaterial und der Matrix bildet.

10. Körper nach Anspruch 9, ferner dadurch gekennzeichnet, daß der stahl aus der aus den Legierungsstählen und den nichtrostenden Stählen bestehenden Gruppe ausgewählt ist.

11. Körper nach einem der Ansprüche 1 bis 10, umfassend: 30 bis 80 Gew.% eines Carbidmaterials mit einer Teilchengröße von mehr als 37 pm, wobei das Carbidmaterial aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählt ist; 20 bis 70 Gew.% eines der aus Stahl, Stahl und Eisen, Stahl und Kupfer, und Stahl und Nickel bestehenden Gruppe ausgewählten Matrixmaterials, dadurch gekennzeichnet, daß das Carbidmaterial mittels pulvermetallurgischer Methoden der Verdichtung und der Diffusionsbindung in festem Zustand in die Matrix eingebettet und an diese gebunden ist.

12. Verfahren zur Herstellung der verschleißfesten Stahl-Hartcarbid-Verbundkörper gemäß einem der Ansprüche 1 bis 8 und 11, umfassend: Das Vermischen von 20 bis 70 Gew.% stahlbildender Pulver mit 30 bis 80 Gew.% Hartcarbidteilchen mit einer Teilchengröße zwischen 8 mm und 37 um unter Bildung eines Gemisches, wobei die stahlbildenden Pulver aus der aus Eisen und Graphit, Legierungsstählen und nichtrostenden Stählen bestehenden Gruppe ausgewählt sind und wobei die Hartcarbidteilchen aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählt sind; das Kaltverpressen des Gemisches unter Bildung einer verdichteten Vorform; und das Verdichten dieser verdichteten Vorform in festem Zustand mittles eines Hochtemperatur- und Hochdruck-Diffusionsbindungs-und -sinterverfahrens, bei dem die verdichtete Vorform bei einer Temperatur oberhalb von 1038°C und unterhalb der Solidustemperatur des Stahls in festem Zustand gesintert wird, um die durch untereinander verbundene Poren gebildete Porosität in der Vorform zu minimieren, und bei dem die Vorform bei einem Druck oberhalb von 689,5.10⁵ Pa und bei einer Temperatur zwischen 871°C und der Schmelztemperatur des Stahls dann heißisostatisch in festem Zustand verpreßt wird.

13. Verfahren nach Anspruch 12 zur Herstellung der verschleißfesten Stahl-Hartcarbid-Verbundkörper gemäß einem der Ansprüche 9 bis 11, ferner gekennzeichnet durch Beschichten der Hartcarbidteilchen mit einem metallischen Überzug vor dem Vermischen mit den stahlbildenden Pulvern.

14. Werkzeug, hergestellt nach dem Verfahren gemäß Anspruch 12 oder 13, mit einem Arbeitsende, das einen harten, verschleißfesten Hartmetalleeinsatz aufweist, einem Stahlkörper, einem den Einsatz mit dem Körper verbindenden Bindungsbereich, dadurch gekennzeichnet, daß der Bindungsbereich eine Eisen und Kobalt enthaltende Legierung umfaßt und im wesentlichen frei ist von spröden Doppelcarbiden des Eisens und Wolframs.

15. Werkzeug, hergestellt nach dem Verfahren gemäß Anspruch 12 oder 13, gekennzeichnet durch ein Arbeitsende, das einen harten, verschleißfesten kobaltzementierten Carbideinsatz aufweist, einen Stahlkörper, wobei der Einsatz pulvermetallurgisch an den Körper mittels einer Diffusionszone gebunden ist, die während des Hochtemperatursinterns in festem Zustand unter dem Schmelzpunkt des Stahls gebildet ist, und wobei die Diffusionszone Eisen und Kobalt enthält und im wesentlichen frei ist von spröden Doppelcarbiden des Eisens und Wolframs.

16. Werkzeug, hergestellt nach dem Verfahren gemäß Anspruch 12 oder 13, gekennzeichnet durch ein Arbeitsende, das einen harten, verschleißfesten Hartmetalleinsatz aufweist, wobei der Einsatz 30 bis 80 Gew.% eines aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählten Carbidmaterials und 20 bis 70 Gew.% eines aus der aus Stahl, Stahl und Eisen, Stahl und Kupfer, und Stahl und Nickel bestehenden Gruppe ausgewählten Matrixmaterials umfaßt, sowie durch einen Stahlkörper, wobei der Einsatz pulvermetallurgisch an den Körper mittels einer Diffusionszone gebunden ist, die während des Hochtemperatursinterns in festem Zustand unter der Temperatur gebildet ist, bei der der Stahl-Binder mindestens teilweise flüssig ist, und wobei die Diffusionszone im wesentlichen frei von spröden Doppelcarbiden des Eisens und Wolframs ist.

17. Verwendung des Verfahrens gemäß Anspruch 12 oder 13 zur Herstellung des Hartmetallwerkzeugs gemäß Anspruch 14 oder 15, gekennzeichnet durch Einbetten eines vorgeformten kobaltzementierten Carbideinsatzes in eine vorbesteimmte Stelle eines Gemischs eines stahlbildenden Pulvers, Verfestigen des Pulvers um den Einsatz herum unter Bildung einer Vorform und gegenseitiges Eindiffundieren von Kobalt aus dem Einsatz und Eisien aus dem verfestigte stahlbildenden Pulver, das den Einsatz umgibt, bei einer hohen Temperatur unterhalb der Temperatur, bei der der Stahl mindestens teilweise flüssig ist, und gleichzeitig bei einem hohen Druck, unter Ausbildung einer metallurgischen Bindung zwischen dem Einsatz und dem Stahl.

18. Verwendung des Verfahrens gemäß Anspruch 12 oder 13 zur Herstellung des Hartmetallwerkzeugs gemäß Anspruch 16, gekennzeichnet durch Einbetten eines vorgeformten hartmetalleinsatzes in eine vorbestimmte Stelle eines Gemischs eines stahlbildenden Pulvers, wobei der vorgeformte Hartmetalleinsatz 30 bis 80 Gew.% eines aus der aus Wolframcarbid, Titancarbid, Tantalcarbid, Niobcarbid, Zirkoniumcarbid, Vanadiumcarbid, Hafniumcarbid, Molybdäncarbid, Chromcarbid, Borcarbid, Siliciumcarbid, deren Gemischen, deren festen Lösungen und deren zementierten Verbundstoffen bestehenden Gruppe der Hartcarbide ausgewählten Carbidmaterials und 20 bis 70 Gew./ eines aus der aus Stahl, Stahl und Eisen, Stahl und Kupfer, und Stahl und Nickel bestehenden Gruppe ausgewählten Matrixmaterials umfaßt, sowie durch Verfestigen des stahlbildenden Pulvers um den vorgeformten Einsatz herum unter Bildung eine Vorform, Sintern der Vorform in festem Zustand bei einer Temperatur im Bereich von 1038 bis 1232°C und gleichzeitig bei einem Druck oberhalb von 689,5·105 Pa unter Bildung einer metallurgischen Bindung zwischen dem Einsatz und dem Stahl.

## Revendications

1. Corps composite résistant à l'usure, de carbure dur et d'acier, fritté à l'état solide, comprenant 30 à 80% en poids d'un matériau à base de carbure ayant une dimension supérieure à 37 pm, le matériau à base de carbure étant choisi dans le groupe des carbures durs comprenant le carbure de tungstène, le carbure de titane, le carbure de tantale, le carbure de niobium, le carbure de zirconium, le carbure de vanadium, le carbure de hafnium, le carbure de molybdène, le carbure de chrome, le carbure de bore, le carbure de silicium, leur mélanges, leurs solutions solides et les éléments composites frittés formés avec eux, 20 à 70% en poids d'un matériau formant un liant choisi dans le group qui comprend l'acier, l'acier et le fer, l'acier et le cuivre, et l'acier et le nickel, le matériau à base de carbure étant enrobé dans le liant et lié à celui-ci, et une interface formée entre le matériau à base de carbure et le liant et ayant une épaisseur qui ne dépasse pas 5 microns, l'interface étant pratiquement dépourvue de carbures doubles fragiles.

2. Corps selon la revendication 1, caractérisé en outre en ce que l'interface a une épaisseur comprise entre 0 et 40 pm.

3. Corps selon la revendication 1, dans lequel le matériau à base de carbure est un élément composite fritté ayant un liant de cobalt, et caractérisé en outre en ce que l'interface a du fer et du cobalt et une épaisseur de 0 à 40 pm.

4. Corps selon la revendication 3, caractérisé en outre en ce que l'élément composite fritté contient du carbure de tungstène.

5. Corps selon la revendication 1, caractérisé en outre en ce que le carbure dur est le carbure de tungstène.

6. Corps selon la revendication 1, caractérisé en outre en ce que le corps est ductile à température ambiante.

7. Corps selon l'une quelconque des revendications 1, 3 et 5, caractérisé en outre en ce que l'acier est un acier allié.

8. Corps selon l'une quelconque des revendications 1, 3 et 5, caractérisé en ce que l'acier est un acier inoxydable.

9. Corps composite résistant à l'usure à base de carbure dur et d'acier, fritté à l'état solide, contenant 30 à 80% en poids d'un matériau à base de carbure ayant une dimension supérieure à 37 pm et ayant un revêtement métallique, le matériau à base de carbure étant choisi dans le groupe des carbures durs formés du carbure de tungstène, du carbure de titane, du carbure de tantale, du carbure de niobium, du carbure de zirconium, du carbure de vanadium, du carbure de hafnium, du carbure de molybdène, du carbure de chrome, du carbure de bore, du carbure de silicium, de leurs mélanges, de leurs solutions solides et des éléments composites frittés formés à partir d'eux, 20 à 70% en poids d'un matériau formant liant choisi dans le groupe quie comprend l'acier, l'acier et le fer, l'acier et le cuivre, et l'acier et le nickel, le revêtement métallique formant une liaison tenace et adhérente entre le matériau à base de carbure et le liant.

10. Corps selon la revendication 9, caractérisé en outre en ce que l'acier est choisi dans le groupe formé des aciers alliés est des aciers inoxydables.

11. Corps selon l'une quelconque des revendications 1 à 10, contenant 30 à 80% en poids d'un matériau à base de carbure ayant une dimension supérieure à 37 pm, le matériau à base de carbure étant choisi dans le group des carbures durs comprenant le carbure de tungstène, le carbure de titane, le carbure de tantale, le carbure de niobium, le carbure de zirconium, le carbure de vanadium, le carbure de hafnium, le carbure de molybdène, le carbure de chrome, le carbure de bore, le carbure de silicium, leurs mélanges, leurs solutions solides et les éléments composites frittés les contenant, 20 à 70% en poids d'un matériau formant un liant choisi dans le groupe constitué par l'acier, l'acier et le fer, l'acier et le cuivre, et l'acier et le nickel, caractérisé en ce que le matériau à base de carbure est enrobé dans le liant et lié à celui-ci par les techniques de la métallurgie des poudres comprenant une compression et une liaison par diffusion à l'état solide.

12. Procédé de fabrication des corps composites résistant à l'usure à base de carbure dur et d'acier selon l'une quelconque des revendications 1 à 8 et 11, comprenant 1 mélange de 20 à 70% en poids de poudres destinées à former de l'acier avec 30 à 80% en poids de particules de carbure dur ayant une dimension particulaire comprise entre 8 mm et 37 pm afin qu'un mélange soit formé, les poudres destinées à former de l'acier étant choisies dans le groupe comprenant le fer et le graphite, les aciers alliés et les aciers inoxydables, les particules de carbure dur étant choisies dans le groupe des carbures durs comprenant le carbure de tungstène, le carbure de titane, le carbure de tantale, le carbure de niobium, le carbure de zirconium, le carbure de vanadium, le carbure de hafnium, le carbure de molybdène, le carbure de chrome, le carbure de bore, le carbure de silicium, leurs mélanges, leurs solutions solides et les éléments composites frittés les contenant, la compression à froid du mélange sous forme d'une ébauche comprimée, et la densification à l'état solide de l'ébauche comprimée par une opération de frittage et de liaison par diffusion à température élevée et à pression élevée, comprenant un frittage à l'état solide de l'ébauche comprimée à une température supérieure à 1038°C et inférieure à la température de solidus de l'acier afin que la porosité inter- connectée dans l'ébauche soit minimale, puis la compression isostatique à chaud à l'état solide de l'ébauche à une pression supérieure à 689,5.10⁵ Pa et à une température comprise entre 871°C et la température de fusion de l'acier.

13. Procédé selon la revendication 12, destiné à la fabrication de corps composites résistants à l'usure à base de carbure dur et d'acier selon l'une quelconque des revendications 9 à 11, caractérisé en outre par le revêtement des particules de carbure dur par un revêtement métallique avant le mélange avec les poudres destinées à former de t'acier.

14. Outil fabriqué par le procède de la revendication 12 ou de la revendication 13, comprenant une extrémité de travail ayant un élément rapporté de carbure dur fritté résistant à l'usure, un corps contenant de l'acier, une région de liaison reliant l'élément au corps, caractérisé en ce que la région de liaison contient un alliage ayant du fer et du cobalt et étant pratiquement dépourvu de carbures doubles fragiles de fer et de tungstène.

15. Outil fabriqué par le procédé de la revendication 12 ou de la revendication 13, comprenant une extrémité de travail ayant un élément rapporté de carbure fritté par du cobalt, dur et résistant à l'usure, un corps contenant de l'acier, l'élément rapporté étant lié par les techniques de la métallurgie des poudres au corps par une zone de diffusion formée pendant un frittage à l'état solide à température élevée, mais inférieure à la température de fusion de l'acier, la zone diffusée ayant du fer et du cobalt et étant pratiquement dépourvue de carbure double fragile de fer et de tungstène.

16. Outil selon la revendication 12 ou la revendication 13, comprenant une extrémité de travail ayant un élément rapporté de carbure fritté dur et résistant à l'usure, l'élément rapporté contenant 30 à 80% en poids d'un matériau à base de carbure choisi dans le groupe des carbures durs qui comprend le carbure de tungstène, le carbure de titane, le carbure de tantale, le carbure de niobium, le carbure de zirconium, le carbure de vanadium, le carbure de hafnium, le carbure de molybdène, le carbure de chrome, le carbure de bore, le carbure de silicium, leurs mélanges, leurs solutions solides et les éléments composites frittés les contenant, et 20 à 70% en poids d'un matériau formant liant choisi dans le groupe qui comprend l'acier, l'acier et le fer, l'acier et le cuivre, et l'acier et le nickel, un corps contenant de l'acier, l'élément rapporté étant lié par les techniques de la métallurgie des poudres au corps par une zone de diffusion formée pendant le frittage à l'état solide, à température élevée mais inférieure à la température à laquelle le liant d'acier est au moins partiellement liquide, la zone de diffusion étant pratiquement dépourvue de carbures doubles fragiles de fer et de tungstène.

17. Application du procédé selon la revendication 12 ou la revendication 13, destiné à la formation d'un outil de carbure fritté selon la revendication 14 ou la revendication 15, caractérisé par l'enrobage d'un élément rapporté lié par du cobalt, ayant des dimensions prédéterminées, à un emplacement prédéterminé dans un mélange d'une poudre dèstinée à former de l'acier, la consolidation de la poudre autour de l'élément rapporté afin qu'une ébauche soit formée, et la diffusion mutuelle du cobalt de l'ébauche et du fer de la poudre consolidée des éléments destinés à former du fer, à proximité de l'élément rapporté, à une température élevée inférieure à la température à laquelle l'acier est au moins partiellement liquide, et, simultanément, la formation d'une liaison métallurgique entre l'élément rapporté et t'acier, à une pression élevée.

18. Application du procédé selon la revendication 12 ou la revendication 13, destiné à former l'outil de carbure fritté selon la revendication 16, comprenant l'enrobage d'un élément rapporté de carbure fritté ayant des dimensions prédéterminées à un emplacement prédéterminé dans un mélange d'une poudre destinée à former de l'acier, l'élément rapporté de carbure fritté ayant des dimensions prédéterminées contenant 30 à 80% en poids d'un matériau à base de carbure choisi dans le groupe des carbures durs qui comprend le carbure de tungstène, le carbure de titane, le carbure de tantale, le carbure de niobium, le carbure de zirconium, le carbure de vanadium, le carbure de hafnium, le carbure de molybdène, le carbure de chrome, le carbure de bore, le carbure de silicium, leurs mélanges, leurs solutions solides et les éléments composites frittés les contenant, et 20 à 70% en poids d'un matériau formant liant choisi dans le groupe qui comprend l'acier, l'acier et le fer, l'acier et le cuivre, et l'acier et le nickel, la consolidation de la poudre destinée à former de l'acier autour de l'élément rapporté ayant les dimensions prédéterminées afin qu'une ébauche soit formée, le frittage à l'état solide de l'ébauche, à une température comprise entre 1038 et 1232°C et simultanément à une pression supérieure à 689,5,10⁵ Pa afin qu'une liaison métallurgique soit formée entre l'élément rapporté et l'acier.
